

March 12, 1940.

P. H. BUXTON

2,193,245

AMMUNITION

Filed Sept. 16, 1936

Fig. 1.



Fig. 2.



Fig. 3.



Fig. 4.



Fig. 5.



Inventor  
Paul H. Buxton  
W. W. Brumage and Lester Hand  
His Attorneys.

## UNITED STATES PATENT OFFICE

2,193,245

## AMMUNITION

Paul H. Buxton, Alton, Ill., assignor to Western Cartridge Company, East Alton, Ill., a corporation of Delaware

Application September 16, 1936, Serial No. 101,029

4 Claims. (Cl. 29—1.3)

This invention relates generally to ammunition and particularly to metallic cases as employed in ammunition.

In ammunition such, for instance, as shot shells, it is customary to provide a metallic head, usually of brass, into which is fitted and anchored a tube, generally of paper, so as to provide a case into which is loaded the propellant and projectile charges together with a suitable primer. Likewise in ammunition, such as metallic small arms ammunition, a metallic case adapted to contain the primer and the propellant charges and connect with the projectile is provided. Heretofore such cases have generally been made of brass or other copper alloy.

The object of the present invention, generally stated, is to provide an improved ammunition case and round.

A further object of the present invention is to provide a process of manufacturing ammunition cases in which steel may be employed.

A more specific object of this invention is to provide an ammunition case of greater strength and of less weight than those heretofore employed without sacrificing any of the advantageous features of the ammunition cases heretofore constructed.

Other objects will become apparent to those skilled in the art when the following description is read in connection with the accompanying drawing which illustrates the respective steps in a process of manufacturing ammunition cases in accordance with the present invention.

Figure 1 is a perspective view of a sheet metal blank from which the ammunition case is fabricated.

Figure 2 is a perspective view, part being in section showing a cup resulting from drawing operations performed upon the blank of Figure 1.

Figure 3 is a perspective view partly in section showing the result of a further deforming operation upon the cup of Figure 2.

Figure 4 is a view in side elevation of a shot shell case provided with the metallic head shown in Figure 3.

Figure 5 is a perspective view partly in section showing a loaded shot shell.

In accordance with the present invention, generally stated, ammunition cases are formed of steel having such characteristics as to permit them to withstand deep drawing and deformation. The present invention further contemplates a round of ammunition provided with a steel case, rust proofed in such a manner as to withstand deformation after the rust proofing operation.

In accordance with the present invention a steel is selected which will lend itself to the drawing operations required for the production of the ammunition case desired. While in the specific embodiment to be herein described the invention will be described in connection with the manufacture of shot shells, it is to be understood that the features of the invention are also applicable to the manufacture of other ammunition cases, such for instance as metallic small arms ammunition cases, both center fire and rim fire as well as to the manufacture of ammunition cases for ordnance.

While a variety of steels may be employed for the manufacture of ammunition cases, in accordance with the present invention a steel whose physical properties are substantially uniform in all directions is desirable. For example, the ordinary steel employed by ammunition manufacturers, such as the "reenforce" in shot shells, may be employed for the manufacture of ammunition cases where such steel is of a character such as to permit it to be drawn to a reduction of about fifty percent or more. While a reduction of fifty percent is sufficient for the manufacture of shot shell heads for ordinary shot shells in which the metallic head heretofore employed has been relatively short, those shot shells which are provided with a propellant charge, such as to produce higher pressures and higher velocities of the projectile charge, and in which the metallic head has customarily been made about  $\frac{3}{4}$ " long may best be produced from steel whose drawing properties permit greater than 50% reduction. As an example of the steels which may be employed for the manufacture of ammunition cases such as shot shell heads (short or long) and small arms ammunition cases (rim fire or center fire) steels made according to the disclosure of the copending application of Norman P. Goss, Serial No. 41,432, filed on or about September 20, 1935, may be employed with advantage. Four examples of such a steel are given in the following tables showing the analyses thereof, it being understood that the balance in each instance is iron.

|   | Carbon   | Phosphorus | Manganese | Sulphur  | Silicon  |  |
|---|----------|------------|-----------|----------|----------|--|
|   | Per cent | Per cent   | Per cent  | Per cent | Per cent |  |
| 1 | .11      | .012       | .43       | .024     | .02      |  |
| 2 | .06      | .011       | .37       | .029     | .02      |  |
| 3 | .10      | .013       | .43       | .024     | .02      |  |
| 4 | .05      | .010       | .36       | .029     | .02      |  |

Each of the steels whose composition is given

5

10

20

25

30

35

40

45

50

55

in the foregoing table is characterized by the absence of directional properties, that is to say, the physical properties including tensile strength, yield point, elongation, etc. are substantially the same, regardless of the direction in which the reading is taken. For instance, as shown in the following table, the physical properties in a longitudinal direction are substantially the same as the physical properties in the transverse direction for each sample.

|    |                    | Yield point | Tensile strength | Elongation | Erichsen values |
|----|--------------------|-------------|------------------|------------|-----------------|
| 15 |                    |             |                  |            | <i>Per cent</i> |
| 1  | {Longitudinal..... | 41,565      | 55,510           | 32         | 895-900         |
|    | {Transverse.....   | 41,405      | 57,410           | 35.5       |                 |
| 2  | {Longitudinal..... | 36,475      | 49,205           | 37         | 900-905         |
|    | {Transverse.....   | 36,555      | 50,200           | 22         |                 |
| 3  | {Longitudinal..... | 43,370      | 53,410           | 35         | 935-945         |
|    | {Transverse.....   | 46,115      | 55,350           | 39.5       |                 |
| 20 | {Longitudinal..... | 38,240      | 47,050           | 39         | 945-950         |
|    | {Transverse.....   | 42,290      | 49,175           | 31         |                 |

Since the explosive shock to which an ammunition case is subjected in use is such that adequate strength must be provided in all directions, the use of such non-directional steel has the advantage of permitting the employment of lighter gauge stock than would be required with ordinary steel, without, however, sacrificing safety because the tensile strength of thin non-directional steel may be greater than the tensile strength in the weaker direction of heavier steel. Although the tensile strength, in the stronger direction of the heavier steel weight exceeds the tensile strength of the non-directional steel such excess tensile strength is of no utility in ammunition cases. Accordingly, the use of such non-directional steel permits the ammunition cases for a given lead to be made thinner than with directional steel.

40 In order to facilitate drawing of the metal a plating of a lubricating metal, such as copper, cadmium, zinc, etc., may be applied to the sheets of steel before the drawing operation is begun. Blanks formed of the steel above described, may 45 then be passed through a convenient number of drawing dies so as to cold-draw the blanks to cup shape and finally deform the same to the shape desired for the ammunition case. The thickness of the sheet metal from which the blanks are 50 punched will, of course, depend upon the character of ammunition in which it is to be employed. In the case of ordinary shot shells the metal from which the heads may be formed may, for instance, be about .015" thick, while, if the 55 heads are to be employed for high velocity shot shells, heavier gauges, such for instance as .0175" may be employed. In the case of the ordinary shot shells in which short metallic heads are customarily employed reduction of 40%, or even 60 less, is sufficient for the production of suitable heads, while in the case of higher velocity shells where the heads are customarily longer, it is desirable to employ a metal capable of withstanding a reduction of 50 to 65%.

65 When a steel which will withstand the reductions above suggested is employed in the manufacture of ammunition cases, the metal may be cold worked through the drawing and deforming operations to produce the desired case without 70 intermediate heat treating, but it will be understood, of course, that after the drawing and deforming operations are completed it is desirable to anneal the case under such conditions as to release the internal strains which have been set 75 up therein during the cold working. In the case

of the steels mentioned specifically hereinabove, such a strain-relieving anneal may, for example, consist in treating shot shell heads at a temperature of approximately 475° C. for a period of about ten minutes. Such a treatment, while 5 sufficient to relieve the internal strains in the shot shell heads is, nevertheless, not such a heat treatment as will substantially soften or take the stiffness out of the article produced or any part thereof. This represents an advantageous feature in ammunition cases, such as shot shell heads or center fire metallic ammunition cases, in which there are one or more projections upset in the center of the head which are later to be somewhat deformed so as to snugly engage a battery 15 cup to be inserted therein or anchored with the base wad in a shot shell. In the case of shot shells the prongs which are customarily upset for penetration into the base wad have a stiffness in excess of the stiffness provided by the ordinary 20 brass shot shell head and consequently a more secure anchor with the base wad and adjoining parts is achieved by the use of steel treated as hereinbefore described.

Referring now particularly to the drawings 25 which illustrate the product resulting from the various steps in the process of manufacturing an ammunition case in accordance with the present invention, it will be understood that a sheet of metal, such, for instance, as the steel 30 hereinbefore specifically described, and having a thickness of .0175" may be provided. Such a sheet of metal may be given a lubricating plating of copper in any suitable manner. Blanks of the desired size may then be stamped from the sheet 35 so as to provide a disc 1 in the form generally illustrated in Figure 1.

The disc 1 may then be passed through a series of drawing dies in order to fold and draw the disc 1 to the cup shape illustrated in Figure 2 40 wherein the article will be provided with a head section 2 and a flange section 3. In the drawing operation the metal in the flange section 3 may be reduced from the initial thickness of, for instance .0175" to about .006-7" at the open end 45 of the cup.

The cup may then be further cold worked with the usual apparatus for forming crimp 4 at the juncture of the head and flange sections of the cup. The head 2 of the cup may then be centrally upset in order to provide the usual prongs 5 extending upwardly on the interior thereof for the purpose of anchoring with the base wad and adjacent parts later to be inserted. The usual knurling and crimping operations may then be 55 performed upon the flange part 3.

The shot shell head thus produced may then be subjected to the annealing treatment, mentioned above, for the purpose of relieving the internal strains in the article, and thereafter 60 may be rust proofed in any suitable manner which will withstand a further deforming operation at the time of heating. For instance, a further plating of a rust proofing metal may be applied thereto, particularly advantageous results being accomplished by the use of a metal which is electropositive as to iron, such as cadmium or zinc. By the use of metals electropositive to iron, a firmly adhering plating is accomplished both inside and outside of the head and 65 the head will withstand further deformation to which it is customarily subjected during the so-called "heading" operation.

The shot shell head thus produced may then be assembled with the usual paper tube 6, the 75

customary base wad and a suitable primer inserted, and the crimp 4 compressed, as shown in Figure 4, by the action of the bunter customarily employed for carrying out this operation. The 5 assembled shell may then be loaded with a propellant charge 7 and a projectile charge 8 interposed by a suitable wadding 9 so as to form the completed shell.

By the use of steel which is substantially devoid of directional properties, as hereinbefore described, ammunition cases having superior strength to similar cases made of copper alloy may be provided and ammunition cases formed in this manner are particularly preferable for 5 use in worn guns wherein the chamber, because of long use, may have become enlarged to an extent such that an ordinary brass or copper alloy ammunition case might rupture when fired therein. By the use of a steel capable of relatively deep drawing, as hereinbefore described, and characterized by the fact that its physical properties in each direction are substantially the same, an ammunition case may be provided in which, without increasing the thickness of the 10 metal and in fact in many cases by reduction of it, higher pressures may be withstood in worn gun chambers than is possible with the customary copper alloy ammunition cases.

While the present invention has been described 0 with particular reference to its advantages and to the procedure employed in the manufacture of shot shell heads, it is to be understood that the invention is not limited to use in shot shell heads, but that it is of wider applicability since small 5 arms metallic ammunition cases may be manufactured in accordance with the present invention with suitable modifications of the tools employed in the manufacture of the usual copper alloy cases as by appropriate alteration of tolerance and clearance for the working of the different metals. It is to be distinctly understood, therefore, that the present invention is not limited to the precise details of procedure which have hereinbefore been described, but that modifications may be made therein, and that the use 10 of various individual features and subcombina-

tions of features may be made without departing from the spirit of the present invention. It is to be understood, therefore, that such modifications and the use of such individual features and subcombinations of features as present themselves to those skilled in the art, although not specifically described herein, are contemplated by and within the scope of the appended claims. 15

Having thus described the invention, what is claimed is:

1. In the art of making ammunition cases, the process comprising, providing a disc of steel whose physical properties in all directions are substantially uniform, cold drawing the disc to cup shape without heat treating, puncturing the 10 head of the cup to form prongs, and thereafter annealing the cup under conditions such as to relieve the strains therein.

2. In the art of making ammunition cases, the process comprising, providing a disc of steel 20 whose physical properties in all directions are substantially uniform, cold drawing the disc to cup shape, upsetting the head of the cup to form a projection on the interior of the cup, and otherwise deforming the cup all without heat 25 treating; and thereafter annealing the cup to an extent sufficient to relieve the strains therein without substantially softening the metal in the upset projection.

3. In the art of making ammunition cases, the 30 process comprising, providing a disc of steel whose physical properties in all directions are substantially uniform, cold drawing the disc to cup shape without heat treating, and thereafter annealing the cup under conditions such as to 35 relieve the strains therein.

4. In the art of making ammunition cases, the process comprising, providing a disc of steel 40 whose physical properties in all directions are substantially uniform, cold drawing the disc to cup shape, and otherwise deforming the cup all without heat treating; and thereafter annealing the cup to an extent sufficient to relieve the strains therein.

PAUL H. BUXTON.